

Patented Nov. 3, 1925.

1,559,963

# UNITED STATES PATENT OFFICE

FRIEDRICH HEÜSLER, OF DILLENBURG, GERMANY, ASSIGNOR TO THE FIRM OF ISABELLENHÜTTE GESELLSCHAFT MIT BESCHRÄNKTER HAFTUNG, OF DILLENBURG, GERMANY.

## TREATMENT OF COPPER ALLOYS.

No Drawing.

Application filed August 29, 1921. Serial No. 496,600.

To all whom it may concern:

Be it known that I, FRIEDRICH HEÜSLER, a citizen of the German Republic, and residing at Dillenburg, Germany, have invented certain new and useful Improvements in and Relating to the Treatment of Copper Alloys (for which I filed an application in Germany, April 10, 1920), of which the following is a specification.

10 This invention relates to the results of investigations of magnetic alloys previously invented consisting of manganese, copper and aluminum. Some of these alloys can be rolled and forged and I have found that

15 the qualities of copper-alloys of this kind containing from about 10 to 15% of manganese, and from about 7 to 10% aluminum can be completely changed as regards the limit of elasticity and their hardness and

20 cutting power, by prolonged heating.

This invention therefore consists in treating copper alloys with manganese and aluminum contents by heating for a prolonged period to a temperature below red

25 heat for example from about 200 to 250° C. For example an alloy consisting of from 10 to 15% manganese and from 10 to 15% aluminum, the remainder being copper when rolled, annealed and cooled in water, showed a tensile strength of 66 kg. per

30 sq. mm. and an extension of about 21%. The same alloy when treated in the above manner and then subjected for twenty hours to a temperature of 195° showed a tensile

35 strength of 75 kg. per sq. mm. and an extension of 9%. Again the same alloy after being rolled, annealed and cooled and subjected to a temperature of 220° for 10 hours showed a tensile strength of 96 kg. per sq.

40 mm. and an extension of 0%. This hardening or tempering process increases the cutting capacity of the metal so as to render the alloy particularly suitable for the manufacture of knives and more particularly of

45 fruit knives.

It might be expected that this hardening process could be applied to all rolled copper alloys, but by the experiment it has been found that copper alloys containing 13 to 14% manganese, but free from aluminum do not alter with the above treatment, neither do copper alloys containing 13% of manganese and 4 to 5% of aluminum. A copper alloy containing only 5% of manganese and 9% of aluminum was found after

a prolonged exposure at 255° to have had its tensile strength very considerably increased although there was no diminution in the extension. For example such an alloy when forged and cooled from a dark red heat showed an elastic limit of 32 kg., a tensile strength of 77 kg. and an extension of 15%. The same alloy similarly treated and then subjected for twenty hours to a temperature of 255° showed an elastic limit from 46 to 50 kg., a tensile strength of 77 kg. and a extension of 15%. Again the same alloy treated as above described and subjected for 50 hours to a temperature of 255° showed an elastic limit of 50 kg., a tensile strength of 75 kg. and an extension of 16%. An alloy containing from 4 to 5% manganese and only 4 to 5% aluminum is not similarly affected by such heat treatment. During experiments it was found that alloys free from manganese and consisting of 60.5% copper, 37.6% zinc, 1.3% lead, and 0.6% iron or 66% copper, 33.7% zinc and 0.3% iron, after being rolled, annealed and cooled could not be perceptibly hardened. On the other hand similar alloys containing manganese behave in a totally different manner, for example a compressed manganese brass consisting of 57.6 copper, 37.3 zinc, 2.7% manganese and 1.2% aluminum and the remainder iron and lead can be hardened at a temperature of 250°. Such an alloy showed after annealing to 550° C. and cooling, a Brinell hardness of 150. The same alloy after annealing and cooling as above, and after being subjected to heating for twenty four hours at 250° showed a hardness of 163. Again this alloy when annealed at 500° and cooled showed a Brinell hardness of 144, whereas, when further subjected to twenty four hours heating at 250° the hardness was 161. The same alloy after annealing at 450° and cooling, showed a Brinell hardness of 143, but after being subjected to 24 hours heating at 250° showed a Brinell hardness of 160.

The hardening effect is much more marked in the case of brass alloys containing a high proportion of manganese. Such an alloy consisting of 9% manganese, 51% copper and 40% zinc, can be rolled at a high temperature and after forging and annealing at 600° and cooling showed a tensile strength of 54 kg. per sq. mm., an exten-

sion of 11% and a hardness of 166. After heating for 36 hours to 230°, the tensile strength was 60 kg. per sq. mm., an extension of 2% and a hardness of 260. It is also possible to harden alloys containing manganese, copper and tin. An important result, which can be obtained with the use of my invention is that the hardening of manganese, silicon and copper alloys may be effected by temperatures of about 200 to 400° and such alloys may be used to replace the expensive tin-alloys used for bearing-liners.

The following contains some examples of alloys suitable for this purpose.

An alloy consisting of 80.9% of copper, 15% manganese, 2% of iron and 2.1% of silicon, after being forged and annealed at 525° and cooled has a hardness of 195, and after exposure for 24 hours to a temperature of 215° has a hardness of 205, and after this treatment for 60 hours, the hardness of 274.

An alloy consisting of 81% of copper, 14% manganese, 2% iron and 3% silicon cast in sand, shows a hardness of 117, and after exposure for 36 hours at a temperature of 215° has a hardness of 152, and after this treatment for 96 hours, the hardness was 174.

An alloy consisting of 80.6% of copper, 15% manganese, 1% iron and 3.4% silicon, after being forged and annealed at 600° and cooled, has a hardness of 178, and after exposure for 36 hours at a temperature of 215° the hardness of 249.

An alloy consisting of 77% of copper,

14% manganese, 3% iron and 6% silicon, cast in sand, shows a hardness of 170, and after exposure for 24 hours at a temperature of 215° has a hardness of 222, and after this treatment for 60 hours, the hardness was 220.

The essential feature of this invention is not affected by the addition of other metals to the alloys described above, for example iron, nickel, cadmium or lead may be present. The presence of such additions only affects the hardening temperature and in some cases makes the alloys more easily cast.

Now what I claim is:

1. The method of increasing the hardness and elastic limit of alloys containing a predominant proportion of copper and relatively small proportions of manganese and aluminum which consists in subjecting the alloys after they have been cast, rolled or forged, to a prolonged heating treatment at a temperature of approximately 200° C. to 250° C.

2. The method of increasing the hardness and elastic limit of alloys containing a predominant proportion of copper and approximately 10% to 15% manganese, together with approximately 7% to 10% aluminum which consists in subjecting the alloys, after they have been cast, rolled or forged, to a prolonged heating treatment at a temperature of approximately 200° C. to 250° C.

In testimony whereof I have affixed my signature.

DR. FRIEDRICH HEÜSLER.